

May 20, 1952

F. R. REDMAN

2,597,530

METHOD OF TREATING FABRIC

Filed May 1, 1950

5 Sheets-Sheet 1

FIG. 1.



FIG. 1A.



FIG. 2.



FIG. 2A.



FIG. 3.



FIG. 3A.



FIG. 4.



FIG. 4A.



Inventor:  
Frank R. Redman  
by his Attorneys  
Howson & Howson

May 20, 1952

F. R. REDMAN

2,597,530

METHOD OF TREATING FABRIC

Filed May 1, 1950

5 Sheets-Sheet 2

FIG. 5.



FIG. 9.



Inventor:  
Frank R. Redman  
by his Attorneys  
Howson & Howson

May 20, 1952

F. R. REDMAN

2,597,530

METHOD OF TREATING FABRIC

Filed May 1, 1950

5 Sheets-Sheet 3



Inventor:  
Frank R. Redman  
by his Attorneys  
Howdon &  
Howdon

May 20, 1952

F. R. REDMAN

2,597,530

METHOD OF TREATING FABRIC

Filed May 1, 1950

5 Sheets-Sheet 4



Inventor:  
Frank R. Redman  
by his Attorneys  
Howson & Howson

May 20, 1952

F. R. REDMAN

2,597,530

METHOD OF TREATING FABRIC

Filed May 1, 1950

5 Sheets-Sheet 5



## UNITED STATES PATENT OFFICE

2,597,530

## METHOD OF TREATING FABRIC

Frank R. Redman, Yardley, Pa.

Application May 1, 1950, Serial No. 159,296

13 Claims. (Cl. 26—18.5)

1

This invention relates to treatment of tubular knitted fabrics, and more particularly to treatment of such fabrics to prevent or eliminate objectionable shrinkage of garments made therefrom. By a "tubular knitted fabric" is meant one which is knitted in tubular form or one which is knitted in flat form and then converted to tubular form.

This application includes subject matter divided from my copending application Serial No. 55,963, filed October 22, 1948, and is a continuation-in-part thereof.

Shrinkage of a garment occurs upon laundering thereof, and in some instances additional shrinkage may occur upon successive laundering. Shrinkage has long been a problem in the textile industry, and much effort has been directed toward reduction thereof both in woven and knitted fabrics. The problem has been particularly troublesome in the case of knitted fabrics, and in fact shrinkage has prevented use of such fabrics in many fields. Shrinkage of any knitted fabric is due chiefly to stretch thereof during the processing of the fabric, which is necessary to condition it for the making of garments. In the case of tubular knitted fabrics, the fabric undergoes what is known as "wet processing," which includes scouring, bleaching and dyeing. The fabric is knitted in lengths of, for example, one hundred yards and these are fastened together in succession. As the fabric goes through the wet processing in continuous rope form, it is subjected to severe tensional forces lengthwise which impart considerable lengthwise stretch to it, the degree of stretch depending upon the type and weight of the fabric, and also the type and condition of the machinery used in the wet processing. Generally speaking, the fabric may be stretched from a minimum of about 8% to a maximum of about 35% of its length. Thus a lightweight fabric may stretch from 15% to 35%, while a heavyweight fabric, which does not stretch as readily as a lightweight fabric, may stretch from 8% to 15%.

The present invention has for its principal object the provision of a simple, efficient and inexpensive method of treatment of tubular knitted fabric to eliminate objectionable shrinkage thereof.

Another object of the invention is to provide such a method which is applicable to all kinds of tubular knitted fabrics composed of either natural or synthetic fibres.

It has been found that shrinkage of knitted

2

fabric is due to elongation and distortion of the knitted stitches or loops resulting in stretch of the fabric, and to the subsequent return of the stitches to their pre-distortion shape. After a fabric is knitted, and before processing thereof, the stitches have a certain shape and the fabric has certain dimensions. As the fabric goes through the wet processing during which it is in a soft, wet and very elastic state, the stitches are elongated longitudinally and narrowed widthwise due to the tensional forces acting longitudinally or lengthwise of the fabric. Thus the stitches are distorted from the shape they had after knitting and the fabric as a whole is distorted accordingly, being stretched longitudinally and narrowed transversely or widthwise. Upon ordinary drying and other usual treatment such as calendering, the fabric remains in this distorted condition. It might be said that the stitches have acquired a distorted "set" which persists through the usual treatment. Subsequent laundering of a garment made from such a distorted fabric relieves the distorted stitches and causes them to return to their pre-distortion shape, with consequent shortening and widening, i. e. shrinkage, of the garment. The reason for this is that during laundering the yarns are in a wet plastic state and the agitation to which the fabric is subjected in laundering is effective to undo the distorted "set" of the stitches and to permit them to relax to their undistorted shape.

Much effort has been directed toward elimination of shrinkage by special treatment of the fabric prior to the making of garments therefrom. Relaxation drying has been tried but that in itself is ineffective to eliminate shrinkage of tubular knitted fabric caused by the above-mentioned condition. In my prior Patent No. 2,325,544 issued July 27, 1943, there is disclosed and claimed a method which involves relaxation and compressive working of the fibers of the fabric while drying the same, following the wet processing of the fabric. However, it has been found that there is a variation in the results obtained by the said process, as applied to tubular knitted fabrics, due to a wide variation between the knitted stitches. Thus, after treatment of a knitted fabric by the said process, one part of the fabric may have a residual shrinkage of 1%, another part may have a residual shrinkage of 3%, and still another part may have a residual shrinkage of 6%. This causes an undesirable variation between garments, some of which may

be satisfactory, while others are not, from the standpoint of shrinkage.

In order effectively to eliminate shrinkage of garments made from tubular knitted fabric, it is necessary to restore the fabric and its component stitches or loops substantially to the original undistorted condition prior to the making of garments therefrom. I have discovered that this result can be achieved very effectively and inexpensively by expanding the fabric widthwise to a sufficient extent, while allowing sufficient freedom of the fabric lengthwise to enable the widthwise expansion and to permit the yarns of the knitted stitches to "flow" freely or slide over one another, and then releasing the fabric to permit relaxation thereof and return of the stitches to their original undistorted shape. Depending upon the type of fabric, the treatment thereof may be performed while the fabric is wet, moist or dry. For the purpose of this specification, a dry fabric is one that contains only such moisture as it may have absorbed from the air; a moist fabric is one that has been dry and has had moisture added in a content of about 2% to 10% (preferably 3% to 6%) of the weight of the fabric; and a wet fabric is one that has just come from the wet processing, with the excess water removed, the moisture content being about 40% to 85% (preferably 50% to 55%) in excess of the dry condition. While the treatment according to the present invention may be applied to fabric having a moisture content between 10% and 40% in excess of the dry condition, it is not economical to bring the fabric to such a condition either by reducing the moisture content from the wet condition or by increasing the moisture content from the dry condition.

Where a fabric is treated according to the invention either in wet condition or in moist condition, the invention further contemplates drying the fabric after the expansion treatment. In some cases, however, drying is not necessary in the case of moist fabric. Where a fabric to be calendered is treated according to the invention, the invention contemplates calendering of the fabric at any time after the widthwise expansion thereof.

The extent to which the tubular knitted fabric is expanded widthwise, according to the invention, will depend upon the following factors in any instance: the amount of longitudinal stretch present in the fabric; the circumferential dimension at which the fabric was knitted; the character of the fabric as determined by its weight, the number of stitches per unit area, the tightness of knitting, and the size and twist of the yarn; and the condition of the fabric from the standpoint of moisture content.

In practicing the invention, it is readily possible for one skilled in the art to determine the requisite amount of widthwise expansion by inspecting the fabric, using a magnifying glass if necessary, to determine the amount of longitudinal stretch present in the fabric. An alternative procedure is to place marks spaced lengthwise on the fabric before it goes through the wet processing, and measure the elongation of the fabric between the marks after it comes from the wet processing. The other factors above mentioned are either known or are readily determinable, and after a little practice the skilled worker can easily determine the extent to which any particular fabric should be expanded widthwise.

In carrying out the expansion of the fabric, it is most convenient, and therefore preferred, to

expand the tubular fabric substantially in flat condition, and it is therefore convenient to deal with the widthwise expansion in terms of the widthwise dimension to which the flattened tubular fabric should be expanded in order to restore the stitches, upon release of the fabric, to their original undistorted shape.

Reference is now made to the accompanying drawings, wherein:

Figs. 1 to 4 and Figs. 1a to 4a are illustrations, taken from actual photographs, of the various stages through which a fabric passes when treated according to the present invention;

Fig. 5 is a front elevational view of one arrangement which may be employed to carry out the treatment of the fabric when it is performed immediately following wet processing and prior to drying of the fabric;

Fig. 6 is a sectional view taken along line 6-6 of Fig. 5;

Fig. 7 is a fragmentary front view showing the drive employed;

Fig. 8 is a sectional view taken along line 8-8 of Fig. 5;

Fig. 9 is a fragmentary detail view showing more clearly the passage of the fabric over the expanding device;

Fig. 10 is a front elevational view of an arrangement which may be employed when the fabric is treated, according to the invention, after drying thereof; and

Fig. 11 is a sectional view taken along line 11-11 of Figure 10.

Referring first to Figs. 1 to 4, Fig. 1 illustrates within the dot and dash circle a portion of a knitted fabric 10 after knitting thereof and prior to wet processing. As the fabric leaves the knitting machine, the threads or yarns are released and the stitches assume a certain normal shape. This condition is illustrated in Fig. 1 wherein each of the stitches 11 has the shape illustrated, and the fabric is completely free of tension or stretch in any direction. Accordingly, the fabric is entirely free of any distortion, either lengthwise or widthwise, and the stitches or loops are in a state of freedom.

Fig. 2 shows the condition of a portion of the knitted fabric after the wet processing. It will be noted that the stitches 11 are elongated lengthwise or longitudinally of the fabric and they are narrowed widthwise. Due to this condition of the stitches, the fabric as a whole is stretched lengthwise and is narrowed widthwise. As mentioned above, in this condition of the fabric the stitches have acquired a distorted "set" which is not disturbed by ordinary treatment of the fabric such as drying, calendering, etc.

In accordance with the present invention, the tubular fabric is restored to the condition of Fig. 1 by expanding the fabric widthwise—while allowing freedom thereof lengthwise—to such an extent that when the fabric is released, the stitches return to their pre-distortion shape as shown in Fig. 1. Fig. 3 shows the condition of the stitches 11 during the widthwise expansion according to the present invention. It will be noted that the stitches are elongated and distorted widthwise and are narrowed lengthwise, which condition is just the opposite of that shown in Fig. 2. In the transition from the condition of Fig. 2 to that of Fig. 3, the yarns forming the stitches are caused to "flow" past one another, and the condition of Fig. 2 is completely eliminated.

Fig. 4 shows the condition of the fabric fol-

lowing the widthwise expansion thereof, and after the stitches  $11$  are permitted to relax, and the yarns permitted to flow to their original free state. It will be noted that the stitches have returned substantially to the shape they had after knitting, as shown in Fig. 1. Accordingly, the fabric has been restored to its original undistorted condition.

Figs. 1a to 4a are a series of illustrations of a different character showing the steps or stages through which the fabric passes. In these illustrations the dot and dash rectangle represents a portion of a knitted fabric 10a. In Fig. 1a the fabric is shown immediately after knitting thereof and prior to wet processing, as in Fig. 1, and the fabric has been marked to place thereon a representation 12 substantially in the form of a square, with the diagonal dimensions lengthwise and widthwise of the fabric. Fig. 2a shows the same fabric after wet processing, as in Fig. 2, and it will be noted that the square 12 has been distorted so that the lengthwise diagonal dimension has been increased while the widthwise diagonal dimension has been decreased. This indicates longitudinal or lengthwise stretch and widthwise narrowing of the fabric. Fig. 3a shows the fabric during the widthwise expansion treatment according to the present invention, as in Fig. 3. It will be noted that the square 12 is now distorted widthwise, the widthwise diagonal being elongated and the lengthwise diagonal being shortened. Fig. 4a shows the fabric after release thereof, as in Fig. 4, and it will be noted that the square 12 has now assumed substantially its original shape as in Fig. 1a.

As indicated above, the illustrations of Figs. 1 to 4 and Figs. 1a to 4a were taken from actual photographs of tubular knitted fabric treated in accordance with the present invention.

From the foregoing description, it will be understood that the extent of the widthwise expansion of the fabric, as depicted in Figs. 3 and 3a, should be sufficient in any particular instance to cause restoration of the stitches to their original shape when the fabric is released. As previously stated, this will depend upon certain factors, but it is readily possible for one skilled in the art to determine the appropriate extent of expansion on the basis of such factors.

Preferably, the tubular knitted fabric is expanded substantially in flattened form by means of an expanding mechanism over which the tubular fabric is caused to pass, as hereinafter more fully described.

Referring now to Figs. 5 to 9, there is illustrated therein a suitable arrangement for carrying out the invention when the tubular knitted fabric is treated immediately after wet processing and prior to drying. In this arrangement, there is provided a stationary horizontal tubular shell or casing 13 having a longitudinal slot 14 at the front thereof and within which there is rotatably mounted a shaft 15 on one end of which is a sprocket 16 (Fig. 7). This sprocket is connected by means of a driving chain 17 to a sprocket 18 (Fig. 6) which is driven by an electric motor 19 through a gear reduction unit 20. Also mounted on shaft 15 is a V pulley 21 of the self-adjusting type comprising relatively movable flanges which are spring urged toward one another. This pulley is connected through a drive belt 22 to a relatively large V pulley 23 on the shaft 24 of a rotatable drum or roll 25. The belt 22 passes about an auxiliary pulley 26 mounted on a stationary jack screw 27, adjust-

ment of which varies the driving ratio. Associated with the roll or drum 25 is a nip idler roll 28 carried by a support 29 pivoted at 30 and biased by spring means 31. The purpose of this arrangement is to feed the fabric, after treatment according to the present invention, into a dryer represented at 32 which may be of any suitable type. As shown, the roll 25 feeds the fabric 10 onto a conveyor 33 which may be driven at a linear speed less than the peripheral speed of roll 25, so that the fabric is placed on the conveyor in relaxed condition. The present invention is not concerned with the details of the fabric feeding mechanism or the dryer, and the foregoing description will suffice for the present purpose. However, roll 25 serves the additional function of carrying the fabric away from the fabric-expanding mechanism hereinafter described.

Mounted on the stationary horizontal housing 13 are a pair of supports 34 and 35 which are arranged in spaced relation and which carry wheels or rollers 36, 37 and 38, 39. The upper wheels or rollers 36 and 38 are driven from the shaft through gear connections, one of which is visible at 40 in Fig. 6. The gear drives are such that the roller 36 is rotated counter-clockwise, as viewed in Fig. 5, while the roller 38 is rotated clockwise. The lower rollers 37 and 39 are not driven and are simply rotatably carried by the supports 34 and 35.

Associated with the above-described rollers is the mechanism by which the tubular fabric 10 is expanded widthwise in accordance with this invention. In the arrangement shown, such mechanism comprises a pair of roller supporting members 41 and 42 connected to a T-shaped frame 43, at the lower portion of which are provided outwardly extending arms 44 and a circular ring 45. The members 41 and 42 carry lower wheels or rollers 46 and 47, intermediate rollers 48 and 49, and upper rollers 50 and 51. The entire expanding mechanism is supported by virtue of the illustrated association of its rollers 46 to 51 with rollers 36 to 39. A pair of outwardly curved arms 52 and 53 extend upwardly from the frame 43 in association with the supporting members 41 and 42, and these arms carry small rollers 54 and 55 at their upper ends. It will be noted that these rollers extend outwardly slightly beyond the upper rollers 50 and 51.

In operation of the apparatus, the longitudinally-stretched tubular knitted fabric 10 is taken as it comes from the wet processing, while it is still in wet condition, and it is passed upwardly over the ring 45 and over the rollers or wheels on the expanding mechanism, as clearly shown in Fig. 5. As may be seen in Figs. 5 and 9, the fabric passes between the expanding rollers and the driving and supporting rollers carried by the supports 34 and 35. In operation, the rollers 36 and 38 are driven from the shaft 15, as hereinbefore described, and these rollers move the fabric over the expanding mechanism, the fabric traveling upward as indicated by the arrows in Fig. 9. The ring 45 serves to open the tubular fabric in preparation for the expanding treatment, and after leaving said ring, the fabric encounters the expanding rollers, passing over the pairs of spaced rollers 46-47, 48-49 and 50-51 in succession. As the fabric moves to the expanding mechanism, it is free longitudinally or lengthwise so that the yarns may "flow" freely during the expanding operation. Thus the fabric may be deposited beneath said mechanism in a

loosely folded condition so that it is completely free as it moves upward.

The purpose of the small and narrow rollers 54 and 55 is to effect a better flattening of the fabric as it leaves the expanding mechanism and to prevent wrinkling along the edge portions of the flattened fabric. Although the fabric is in flattened condition as it passes over the expanding rolls, such rolls must have substantial thickness, and in the absence of the rollers 54 and 55, there would be a tendency toward wrinkling of the edge portions. The large drum or roll 25, as shown in Fig. 6 moves the fabric upward as it leaves the expanding mechanism and places it on the conveyor 33 as hereinbefore described, and the rollers 54 and 55 place the fabric in better flattened condition for passage between the rolls 25 and 28 and for drying in the drier 32. The roll 25 is driven at a surface speed such that it accepts the fabric as the latter is supplied from the expanding mechanism. To this end, the roll 25 should be driven at such a peripheral speed relative to the peripheral speed of rollers 36 and 38 that the fabric is carried away without exerting tension thereon. Since the widthwise expansion of the fabric shortens it lengthwise, it will be apparent that the peripheral speed of roll 25 must be less than the peripheral speed of rollers 36 and 38.

Referring now to Figs. 10 and 11, there is shown an arrangement which may be employed when it is desired to treat the tubular knitted fabric, according to the present invention, after the fabric has been wet processed and dried in any type of drier. While such treatment is generally an alternative to that illustrated in Figs. 5 to 9, it may be in addition thereto if the fabric has been subjected to any longitudinal tension during drying or handling after the first expanding treatment.

It should be noted here that while cotton and wool fabrics may be treated in various conditions of moisture content as hereinbefore mentioned, some fabrics must be treated after they have been dried from the wet condition. For example, when a fabric is napped it is preferably dry, and the napping stretches the fabric lengthwise by as much as 16%. The napped fabric should not be wet as this would destroy the nap. However, it may be properly moistened and then treated according to the present invention. Fabrics composed of synthetic yarns, such as those composed of nylon or cellulose acetate yarns, may or may not be moistened before treatment according to the invention. In the case of viscose types, moisture is very much preferred.

Referring to the apparatus of Figs. 10 and 11, there is provided an idler roll 56 over which the dry fabric 10 is passed, and from which the fabric passes to a moistening means 57. The latter may be adapted to moisten the fabric in any suitable manner, as by steaming it or subjecting it to a fine water spray. In the arrangement illustrated, an enclosing structure 58 is formed to provide a passageway through which the fabric may pass, and within said structure are transverse spray members 59 and 60 which are supplied with steam or water through a common header 61 from a supply conduit 62. The entire moistening assembly may be supported in any suitable manner, for example by means of rollers 63 and 64 engaging tracks 65 and 66. Of course, in operation, the fabric moistening assembly is stationary.

Below the said assembly is an expanding

mechanism generally similar to that previously described but in inverted position because of the fact that the fabric is traveling downward in this instance. In this instance, a stationary member 5 has mounted thereon supports 34a and 35a which carry idler rollers 36a to 39a for supporting the expanding mechanism. The latter comprises roller-carrying supports 41a and 42a connected to a frame 43a, the assembly comprising these elements being in inverted position with respect to the previously described arrangement. In this instance, the frame 43a includes a loop 67 which extends upward within the moistening enclosure. The tubular fabric passes over this loop and is opened thereby for uniform moistening and in preparation for the expanding treatment.

Below the expanding mechanism is an arrangement 68 which is adapted to pull the tubular fabric over the expanding rolls and feed it, with or without calendering, to a relaxation drier 69 which may be of the character disclosed in my prior Patent No. 2,440,209, issued April 20, 1948. Above the expanding rolls the fabric should be free lengthwise to enable the widthwise expansion and to permit "flow" of the yarns. In most instances, it will be desired to calender the fabric after the expanding treatment, but in the case of napped fabric, calendering is undesirable because it would defeat the purpose of napping. For these reasons, the mechanism 68 is provided with a pair of calendering rolls 70 and 71, and a pair of ordinary feed or nip rolls 72 and 73, arranged for selective use of either pair of rolls. As shown in Fig. 11, the rolls 71 and 73 are rotatably supported on screw supports 74 and 75, and by adjustment of either support, the associated roll may be placed in operative or inoperative position. In the illustration, the roll 71 is in inoperative position, while the roll 73 is in operative position. The rolls 70 and 72 are rotatably supported by individual support means 76 and 77 which include springs for urging the rolls into engagement with the associated rolls. It should be noted that the expanding mechanism not only treats the fabric according to the present invention but also supplies it in flattened condition to the above-mentioned rolls. This is particularly important when the calendering rolls are operative, as it is necessary to supply the fabric thereto in flat condition.

The arrangements hereinbefore described are adapted to treat the fabric in wet or moist condition. Most fabrics are better treated either wet or moist because the moistened fibres are more plastic and elastic, and less resistant to the desired expansion of the fabric, than they are in the dry condition. However, some fabrics may be treated in the dry condition as previously mentioned. In such case, the apparatus of Figs. 10 and 11 may be employed without the moistening means and without the drying means.

With respect to the invention generally, the following are examples of actual practice of the invention.

*Example No. 1*

1 x 1 rib

Yarn count, 20/1CP

Stitches per inch, 28

70 Head size of knitting machine, 15" diameter

14 cut

Fabric stretched (elongated) in wet processing from original length, 14.6%

75 Expanded (wet or moist) in flattened condition to a widthwise dimension of 22½"

## Example No. 2

## Interlock

Yarn count, 36/1C

Stitches per inch, 31-32

Head size of knitting machine, 15" diameter

Fabric stretched (elongated) in wet processing  
from original length, 11.1%Expanded (wet or moist) in flattened condition  
to a widthwise dimension of 22½"

While the invention has been described with reference to certain specific arrangements for carrying out the process of the present invention, and certain specific examples have been given, it is to be understood that the invention is not limited thereto but contemplates the widthwise expansion of tubular knitted fabric, by any suitable means, to an extent to effect restoration of the stitches or loops, upon release of the fabric, substantially to the shape they had immediately after the fabric was knitted.

I claim:

1. A method of reducing shrinkage in tubular knitted fabric which has been elongated lengthwise and narrowed widthwise by processing subsequent to knitting of the fabric, and the stitches of which are distorted lengthwise and widthwise, said method comprising moving the tubular knitted fabric lengthwise through a treatment zone while providing lengthwise freedom of the fabric, internally expanding the tubular fabric widthwise within said zone to effect lengthwise shortening or condensing of the fabric, and permitting the fabric to relax, whereby to effect repositioning of the stitches substantially to their original knitted form and restoration of the fabric substantially to its normal condition.

2. A method of treating tubular knitted fabric according to claim 1, wherein at least at the time the fabric is permitted to relax it contains moisture.

3. A method of reducing shrinkage in tubular knitted fabric which has been elongated lengthwise and narrowed widthwise by processing subsequent to knitting of the fabric, and the stitches of which are distorted lengthwise and widthwise, said method comprising moving the tubular knitted fabric lengthwise through a treatment zone while providing lengthwise freedom of the fabric, internally expanding the tubular fabric widthwise within said zone to effect sliding of the stitch yarns over or past one another and consequent widthwise distention of the stitches, and permitting the fabric to relax, whereby to effect repositioning of the stitches substantially to their original knitted form and restoration of the fabric substantially to its normal condition.

4. A method of reducing shrinkage in tubular knitted fabric which has been elongated lengthwise and narrowed widthwise by processing subsequent to knitting of the fabric, and the stitches of which are distorted lengthwise and widthwise, said method comprising moving the tubular knitted fabric lengthwise in wet condition through a treatment zone while providing lengthwise freedom of the fabric, internally expanding the tubular fabric widthwise within said zone to effect lengthwise shortening or condensing of the fabric, permitting the fabric to relax, whereby to effect repositioning of the stitches substantially to their original knitted form and restoration of the fabric substantially to its normal condition, and drying the fabric in a relaxed state.

5. A method of reducing shrinkage in tubular knitted fabric which has been elongated length-

wise and narrowed widthwise by processing subsequent to knitting of the fabric, and the stitches of which are distorted lengthwise and widthwise, said method comprising moving the tubular knitted fabric lengthwise through a treatment zone while providing lengthwise freedom of the fabric, internally expanding the tubular fabric widthwise within said zone to effect lengthwise shortening or condensing of the fabric, pressing the fabric, and permitting the fabric to relax, whereby to effect repositioning of the stitches substantially to their original knitted form and restoration of the fabric substantially to its normal condition.

15 6. A method of reducing shrinkage in tubular knitted fabric which has been elongated lengthwise and narrowed widthwise by processing subsequent to knitting of the fabric, and the stitches of which are distorted lengthwise and widthwise, said method comprising moving the tubular knitted fabric lengthwise through a treatment zone while providing lengthwise freedom of the fabric, internally expanding the tubular fabric widthwise within said zone to effect lengthwise shortening or condensing of the fabric, calendering the fabric in moist condition, and permitting the fabric to relax, whereby to effect repositioning of the stitches substantially to their original knitted form and restoration of the fabric substantially to its normal condition.

30 7. A method of reducing shrinkage in tubular knitted fabric which has been elongated lengthwise and narrowed widthwise by processing subsequent to knitting of the fabric, and the stitches of which are distorted lengthwise and widthwise, said method comprising moving the tubular knitted fabric lengthwise through a treatment zone while providing lengthwise freedom of the fabric, moistening and internally expanding the tubular fabric widthwise within said zone to effect lengthwise shortening or condensing of the fabric, and permitting the fabric to relax, whereby to effect repositioning of the stitches substantially to their original knitted form and restoration of the fabric substantially to its normal condition.

35 8. A method of reducing shrinkage in tubular knitted fabric which has been elongated lengthwise and narrowed widthwise by processing subsequent to knitting of the fabric, and the stitches of which are distorted lengthwise and widthwise, said method comprising moving the tubular knitted fabric lengthwise at a predetermined speed to an expansion station, moving the fabric from said station at a second predetermined speed sufficiently less than said first speed to permit lengthwise shortening or condensing of the fabric, internally expanding the tubular fabric widthwise at said station to effect lengthwise shortening or condensing of the fabric, and permitting the fabric to relax, whereby to effect repositioning of the stitches substantially to their original knitted form and restoration of the fabric substantially to its normal condition.

65 9. A method of treating tubular knitted fabric according to claim 8, wherein at least at the time the fabric is permitted to relax it contains moisture.

70 10. A method of reducing shrinkage in tubular knitted fabric which has been elongated lengthwise and narrowed widthwise by processing subsequent to knitting of the fabric, and the stitches of which are distorted lengthwise and widthwise, said method comprising supplying the tubular knitted fabric lengthwise to an expansion

11

station, propelling the fabric at said station at a predetermined speed, moving the fabric from said station at a second predetermined speed sufficiently less than said first speed to permit lengthwise shortening or condensing of the fabric, internally expanding the tubular fabric widthwise at said station to effect lengthwise shortening or condensing of the fabric, and permitting the fabric to relax, whereby to effect repositioning of the stitches substantially to their original knitted form and restoration of the fabric substantially to its normal condition.

11. A method of reducing shrinkage in tubular knitted fabric which has been elongated lengthwise and narrowed widthwise by processing subsequent to knitting of the fabric, and the stitches of which are distorted lengthwise and widthwise, said method comprising moving the tubular knitted fabric lengthwise to and from an expansion station while providing lengthwise freedom of the fabric, internally expanding the tubular fabric widthwise at said station to effect lengthwise shortening or condensing of the fabric, and permitting the fabric to relax, whereby to effect repositioning of the stitches substantially to their original knitted form and restoration of the fabric substantially to its normal condition.

12. A method of reducing shrinkage in tubular knitted fabric which has been elongated lengthwise and narrowed widthwise by processing subsequent to knitting of the fabric, and the stitches of which are distorted lengthwise and widthwise, said method comprising moving the tubular knitted fabric lengthwise to and from an expansion station while providing lengthwise freedom of the fabric, internally expanding the tubular fabric widthwise at said station to effect length-

wise shortening or condensing of the fabric, pressing the fabric, and permitting the fabric to relax, whereby to effect repositioning of the stitches substantially to their original knitted form and restoration of the fabric substantially to its normal condition.

13. A method of reducing shrinkage in tubular knitted fabric which has been elongated lengthwise and narrowed widthwise by processing subsequent to knitting of the fabric, and the stitches of which are distorted lengthwise and widthwise, said method comprising moving the tubular knitted fabric lengthwise to and from an expansion station while providing lengthwise freedom of the fabric, internally expanding the tubular fabric widthwise at said station to effect lengthwise shortening or condensing of the fabric, calendering the fabric in moist condition, and permitting the fabric to relax, whereby to effect repositioning of the stitches substantially to their original knitted form and restoration of the fabric substantially to its normal condition.

FRANK R. REDMAN.

## REFERENCES CITED

The following references are of record in the file of this patent:

## UNITED STATES PATENTS

| Number    | Name        | Date          |
|-----------|-------------|---------------|
| 964,088   | Chatfield   | July 12, 1910 |
| 1,280,607 | Widdowson   | Oct. 1, 1918  |
| 1,372,766 | Moore       | Mar. 29, 1921 |
| 1,790,655 | Cohn        | Feb. 3, 1931  |
| 2,011,935 | Kasanof     | Aug. 20, 1935 |
| 2,187,644 | Cohn et al. | Jan. 16, 1940 |
| 2,294,642 | Wedler      | Sept. 1, 1942 |